

March 14, 1944.

R. H. TAYLOR

2,344,066

METHOD OF AND APPARATUS FOR PRODUCING CUTTING AND ABRADING ARTICLES

Filed Aug. 4, 1942

2 Sheets-Sheet 1



INVENTOR  
*Rutherford H. Taylor.*  
BY  
*James G. Bevill*  
ATTORNEY

March 14, 1944.

R. H. TAYLOR

2,344,066

METHOD OF AND APPARATUS FOR PRODUCING CUTTING AND ABRADING ARTICLES

Filed Aug. 4, 1942

2 Sheets-Sheet 2



INVENTOR

*Rutherford H. Taylor.*  
BY  
*James G. Bechler.*  
ATTORNEY

## UNITED STATES PATENT OFFICE

2,344,066

## METHOD OF AND APPARATUS FOR PRODUCING CUTTING AND ABRADING ARTICLES

Rutherford H. Taylor, Millburn, N. J., assignor to J. K. Smit &amp; Sons, Inc., New York, N. Y., a corporation of New York

Application August 4, 1942, Serial No. 453,546

14 Claims.

(Cl. 22—122)

This invention relates to an improved method of producing articles comprising a metal matrix with cutting and abrading particles embedded therein. My invention therefore is useful in a great variety of industries. However, for purposes of this application I have elected to illustrate the same in connection with the making of diamond tools such as rotary drill bits.

In the setting of industrial diamonds in the making of diamond tools, several methods have been employed which while used quite extensively are not entirely satisfactory and require skilled labor. One prior method of setting diamonds in diamond tools is to form depressions in the face of the tool blank, place a diamond in each depression and then with punches and mauls facets are formed about the diamonds to hold them in place. This operation is slow and requires skilled and experienced operators.

Another method heretofore employed involves arranging the diamonds in a mold and while retaining them in position with a plastic, heat and pressure is applied to a mass of powdered metal confined within the mold. This method while workable fails to produce a tool in which the diamonds will be adequately retained in place when the tool is put in service, so that the loss of diamonds is objectionably high.

A still further method which has been employed is to cast a matrix about the diamonds, by arranging the diamonds in the bottom of a mold and pouring molten metal into the mold upon the diamonds. Difficulties have been experienced with this method, however, in holding the diamonds in their proper places during the process of pouring the molten metal, due to "floating" of the diamonds.

The present method and apparatus eliminates the drawbacks and difficulties of the methods above referred to in a very simple, inexpensive and efficient fashion.

Briefly the present invention contemplates introducing molten metal below the diamonds, instead of upon them, and forcing this molten metal upwardly about the diamonds. In this way I at once eliminate the "floating" problem, the skill that is required in the hand setting method above referred to is not required, and I obtain excellent retention of the diamonds in the cast metal matrix as distinguished from the relatively poor results obtained in the powdered metal process, wherein, as above explained, the diamond loss is objectionably high owing to poor retention of the diamonds against dislodgment.

In the accompanying drawings I have illus-

trated one embodiment of my invention in the form of a suitable equipment for the casting of diamond core bits. As above pointed out, however, this apparatus is purely illustrative and not definitive inasmuch as obviously changes may be made therein within the purview of my invention. It is to be understood, also, that the showing of a diamond core bit is for purposes of illustration and description only, inasmuch as my invention obviously may be employed in the manufacture of articles other than diamond core bits.

Fig. 1 is an elevational view of an apparatus suitable for the practice of my invention; and

Fig. 2 is a sectional elevational view of the mold portion of the apparatus of Fig. 1.

Referring to the drawings in detail: 2 designates the base of my improved apparatus. Mounted upon this base is a cupped member or block 3 into which is threaded a cylindrical shell 4 provided exteriorly with electric winding 6. The shell 4 contains a carbon tube or cylinder 8 provided with piston 10, to the upper end of which plunger 12 is secured. As will be brought out hereinafter, the winding 6 is for heating the structure to prevent too sudden cooling of the molten metal during the casting operation.

Mounted upon the top of the structure so far described is a split strap or ring 14 which receives the preformed threaded hollow shank 16 of the bit, the matrix to be cast being united to this shank in the casting operation.

The head 18 of the shank 16 extends upwardly into a mold cavity 20 formed in a block 22 which sits upon the split strap or ring 14 above referred to.

Resting in an annular depression in the top of the mold block 22 is a mold cover plate or die cover plate 24. This cover plate on its lower face is shaped so as to be complementary to the shape desired of the working end of the finished tool. Inasmuch as I have illustrated an apparatus for casting core bits, and inasmuch as the working end or nose of the bit is to be convex, the underside of the plate 24 is concaved, as shown at 26, and this portion of the plate is drilled to provide a series of diamond-receiving holes 28. The pattern of these holes conforms of course to the desired disposition or arrangement of the diamonds in the finished tool.

As above mentioned, the plate 24 is cup shaped, which provides a cavity or chamber 30 at the upper side of the plate.

Extending through the center of the cover plate 24 is a tubular member 32. The lower end of this member is of carbon, for instance, while

its upper portion is of steel and extends through the cover plate 34 of the member 24.

The member 32 functions as a pouring tube for introducing molten metal into the mold cavity below the diamonds which are temporarily attached to the underside of cover plate 24, and also provides the core opening in the finished tool which in this instance happens to be a core bit.

Secured in the base member 2 is a vertically extending post 35, equipped with an arm 36 which is adapted to be swung above the top of the cover plate 34 so as to clamp all parts in position.

Communicating with the lower end of the cylinder 8 is compressed air line 38. This line is equipped with valve 40 which is adapted to be opened and closed by foot pedal 42.

Communicating with the chamber 30 at the top of the mold is suction line 44.

In the casting of a tool I proceed as follows: With the mold cover plate 24 out of the mold and upside down as compared with the showing in the drawings, I dispose the diamonds which are to constitute the cutting elements of the tool in the openings or orifices 28 of the plate. This assembly may then be sprayed with any suitable adhesive, such, for example, as collodion. After the pouring tube 32 has been inserted in the plate and the tool shank 18 has been placed in position, the die plate with the diamonds adhering thereto is inverted and placed in position on the mold body member 22. The cap or cover 34 may now be placed in position and the arm 36 swung into place and tightened down so that the parts are all now in position for casting.

With the circuit to the winding 12 closed the equipment is allowed to stand until it has heated up to say four or five hundred degrees Fahrenheit or to whatever other temperature may be found desirable. The purpose of this heating is to prevent too sudden cooling of the molten metal when it is poured into the mold.

The suction line 44 is now operated to exhaust all cavities of the mold so far as possible thereby to free the same of gases and promote the production of a casting free of blowholes. Suction is preferably maintained throughout the actual casting operation so as to insure the removal of such gases as are evolved during the casting operation. The molten metal may now be poured through the pouring tube 32, entering the mold as above explained beneath the diamonds and almost simultaneously therewith the pedal 42 is operated to open the valve 40 and to admit compressed air to the cylinder 4 beneath the piston 10. This quickly forces the plunger 12 upwardly in the cylinder 8 and hollow tool shank 16 to cause the molten metal to flow into intimate contact with and about the diamonds at the orifices 28 and about the end of the tool shank, to produce a matrix attached to the shank with diamonds embedded in the surface thereof.

It will be appreciated from the foregoing that there is no "floating" problem to contend with in practicing my invention, inasmuch as the diamonds are at the top of the mold and the molten metal is admitted beneath them and then forced upwardly by the plunger 12. I find, furthermore, that this procedure produces a very dense and uniform matrix, free of blowholes and other imperfections, and in which the diamonds are firmly embedded.

It will be apparent from the drawings, that in the finished tool the matrix will be securely affixed or cast to the tool shank 16, the head 18

of the shank being provided with ports 46 into which the molten metal is forced during casting.

In the casting operation some of the molten metal is forced past the diamonds through the orifices 28. This produces fine filaments of metal projecting from the working end of the tool. These are easily broken off and the tool sandblasted or otherwise treated to give it the desired finish.

10 As stated near the outset of this specification, an equipment for producing core bits has been illustrated for purposes of description only, it being very obvious that changes may be made therein for producing the same or other tools 15 without departing from the spirit and scope of my invention.

What I claim is:

1. The method of forming a metal matrix with cutting and abrading particles embedded therein, 20 which method comprises confining the particles in a mold and then introducing molten metal into the mold from beneath the particles.

2. The method of forming a metal matrix having cutting and abrading particles embedded therein, 25 which method comprises confining the particles in the upper part of a mold, introducing molten metal into the mold from beneath the particles and while the metal is still in molten condition applying upward pressure to the same.

3. The method of making diamond tools comprising a metal matrix having diamonds embedded therein, which method comprises temporarily anchoring the diamonds in a mold and then introducing molten metal into the mold from 35 beneath the diamonds while preventing upward movement of the diamonds.

4. The method of making cutting and abrading tools composed of a metal matrix having cutting and abrading particles embedded therein, 40 which method comprises introducing molten metal into the lower part of a covered mold with the cutting and abrading particles held against upward movement by the mold cover.

5. The method of making cutting and abrading tools composed of a metal matrix having cutting and abrading particles embedded therein, 45 which method comprises securing the cutting and abrading particles in the form of an annulus to the underside of the cover plate of a mold, pouring molten metal into the mold through the cover plate within the inner periphery of the annulus and then forcing the molten metal upwardly of the mold and laterally into contact with the cutting and abrading particles.

55 6. The method of making cutting and abrading tools composed of a metal matrix having cutting and abrading particles embedded therein, which method comprises disposing the preformed shank of the tool in the lower part of a mold, 60 disposing the cutting and abrading particles in the upper part of the mold above and spaced from the tool shank, and while retaining the shank and particles against relative movement introducing molten metal into the space between

65 the two for flow about the end of the shank and about the cutting and abrading particles whereby a matrix is formed in which the end of the tool shank and the cutting and abrading particles are embedded.

7. The method of making cutting and abrading tools composed of a metal matrix with cutting and abrading particles embedded therein, which method comprises temporarily adhesively securing the cutting and abrading particles to the underside of the cover plate of a mold, admitting

molten metal into the mold beneath the cutting and abrading particles and applying pressure to the underside of the molten metal mass to force the same to flow upwardly about and in contact with the cutting and abrading particles.

8. An apparatus for molding articles composed of a metal matrix having cutting and abrading particles embedded therein, said apparatus comprising in combination a closed mold having provision for introducing the molten metal, which is to constitute the matrix, into the mold beneath the cutting and abrading particles.

9. An apparatus for molding articles composed of a metal matrix having cutting and abrading particles embedded therein, said apparatus comprising in combination a mold, a plate at the top of the mold cavity to the underside of which the cutting and abrading particles are adapted to be held, means for admitting the metal of the matrix in molten condition to the mold cavity beneath the cutting and abrading particles, and a plunger for exerting upward pressure on the molten mass.

10. An apparatus for molding articles composed of a metal matrix having cutting and abrading particles embedded therein, said apparatus comprising in combination a mold, a plate across the top of the mold cavity to the underside of which cutting and abrasive particles may be held temporarily, means for admitting the metal of the matrix while molten to the mold cavity beneath the cutting and abrading particles, and an air operated plunger for exerting upward pressure on the molten mass to cause the same to flow about and in contact with the cutting and abrasive particles.

11. An apparatus for molding articles comprising a metal matrix with embedded cutting and abrading particles, said apparatus comprising in combination a mold having a plate across the top of the mold cavity, to the underside of which the cutting and abrading particles are adapted to be attached temporarily, a pouring tube through which the matrix metal in molten condition may be poured into the mold cavity beneath the cutting and abrading particles, a plunger below the mold cavity and an air operated piston for forcing said plunger upwardly thereby to

cause the molten metal to flow around and in contact with the cutting and abrading particles.

12. An apparatus for producing cutting and abrading tools comprising a metal matrix and embedded cutting and abrading particles, said apparatus comprising in combination a mold equipped with a perforated plate across the top of the mold cavity to the underside of which plate the cutting and abrasive particles may be attached temporarily, the upper side of said plate being cupped, a cover plate for said cupped portion of the plate, a suction line in communication with the chamber thus formed at the upper side of said perforated plate, and a pouring tube adapted to admit the molten matrix metal to the mold cavity while the cavity is exhausted by said suction means.

13. An apparatus for producing cutting and abrading tools comprising a metal matrix molded to a preformed metal tool shank, the cutting and abrading particles of the tool being embedded in the said matrix, said apparatus comprising in combination a mold into the cavity of which the preformed tool shank is adapted to be projected, a plate across the top of the mold cavity, said plate being perforated and the cutting and abrading particles being adapted to be attached temporarily to the underside of said plate at said perforations, a pouring tube leading into the mold cavity between the tool shank and the said perforated plate so that the molten metal of the matrix may be introduced into the mold cavity beneath the cutting and abrading particles, and an air operated plunger extending into the tool shank for exerting upward pressure on the molten metal to cause the same to flow about the cutting and abrading particles.

14. The method of making cutting and abrading tools composed of a matrix having cutting and abrading particles embedded therein, which method comprises pouring molten metal into a mould cavity beneath the cutting and abrading particles and while restraining the particles against upward movement and while the metal is still in a molten condition imposing upward pressure upon the metal, this pressure being maintained until the metal has solidified.

RUTHERFORD H. TAYLOR.